

Patented Jan. 13, 1942

2,270,181

# UNITED STATES PATENT OFFICE

2,270,181

## MAKING SHAPED ARTICLES FROM COKE AND PITCH

Edward R. Cole and Richard I. Thrune, Midland,  
Mich., assignors to The Dow Chemical Company,  
Midland, Mich., a corporation of Michigan

No Drawing. Application August 12, 1939,  
Serial No. 289,930

6 Claims. (Cl. 106—284)

The invention relates to an improvement in the art of making shaped carbon articles. It relates particularly to an improvement in the manufacture of graphite electrodes.

Shaped carbon articles are customarily made from petroleum coke and pitch. The ingredients are mixed, heated to soften the pitch, and molded or extruded to the desired form and size, and are then baked to carbonize the pitch binder. High temperature baking is known to convert the article to a graphitic form of carbon throughout. Such articles are useful, for example, as electrodes in the manufacture of chlorine and caustic soda from salt brine, or of metals from fused metal chlorides.

A graphite electrode should have as high an apparent density as possible, and as low electrical resistance as possible for most efficient operation and to give the longest useful life from a given electrode weight. Even slight increases in apparent density and correspondingly slight reductions in the electrical resistance of an electrode are of great practical importance. Thus, a change in apparent density from 1.52 to 1.59 is an increase of 5.6 per cent in the mass per unit volume, and indicates an increase in the expected life of the electrode under otherwise equal conditions. Similarly, a decrease in resistance from 0.00034 to 0.00030 ohm per inch cube represents about a 12 per cent electrical savings, in the form of lowered  $I^2R$  loss in the use of the electrode.

It is accordingly among the objects of the invention to provide an improvement in the art of making shaped carbon bodies from coke and pitch, whereby the apparent density is increased over that usually obtained, and the electrical resistance of a graphitized article therefrom is decreased. Another object is to provide a method of increasing the coking power and the melting point of coal-tar pitch without unduly increasing the heat and pressure requirements in making shaped coke-pitch articles therefrom. Yet another object is to provide a method of modifying the properties of pitch so that its adhesiveness or binding power in a coke-pitch mixture is increased, and the extrusion of uniform coke-pitch articles is facilitated.

According to the present invention, coke and pitch, and more particularly calcined petroleum coke and coal-tar pitch, each in the proportion and in the state of fine subdivision usually employed in making coke-pitch mixtures for the preparation of shaped carbon articles, are mixed at or near room temperature with a minor proportion of a polychlorinated hydrocarbon, and preferably from 0.7 to 6 per cent of carbon tetrachloride, or of acetylene tetrachloride, based on the weight of pitch present. The coke-pitch-chloro-hydrocarbon mixture is then heated to a

reaction temperature above the initial melting point of the pitch but below a carbonizing temperature, and mixed at this temperature to provide a uniform composition of the desired consistency for a period suitably in the range from 10 to 45 minutes and preferably between 15 and 30 minutes. The so-treated mixture is cooled and then molded or extruded, and finally heated sufficiently to carbonize the binder or to graphitize the entire body of carbon present. If desired, pitch may be reacted with carbon tetrachloride and then mixed with coke in the usual manner.

Graphite articles formed according to the present improved method have higher apparent density and lower electrical resistance than those prepared without the use of the carbon tetrachloride or equivalent chloro-hydrocarbon. This is believed to be due to a reaction of carbon tetrachloride on pitch at temperatures above the initial melting point of the pitch. This reaction increases the free carbon content, the coking power, and the melting point of the pitch, and decreases to a certain extent the loss due to volatile matter during the carbonizing operation applied to the pitch-coke article. It also increases the adhesiveness of the pitch, and facilitates the extrusion of coke-pitch articles.

The following table illustrates the effect of carbon tetrachloride on pitch. In the reported experiments, the indicated percentage of carbon tetrachloride was mixed with pitch which had an initial melting point of 224° F. (107° C.) and a free carbon content of 29 per cent. The mixture was heated for from 10 to 20 minutes at a maximum temperature, measured in the melt, of from 150°-180° C., the heating bath being held at about 160°-200° C. In each instance, evolution of hydrogen chloride was observed from the pitch-carbon tetrachloride mixture. The melting point of the cooled product and its free carbon content were determined.

Table I

| Sample No. | Per cent $CCl_4$ | Final M. P. | Rise in M. P. | Free carbon | Increase in free carbon |
|------------|------------------|-------------|---------------|-------------|-------------------------|
| 1          | 1                | 117         | 10            | 33.4        | 4.4                     |
| 2          | 1                | 120         | 13            | 38.3        | 9.3                     |
| 3          | 3                | 150         | 43            | 41.6        | 12.6                    |
| 4          | 3                | 152         | 45            | 41.7        | 12.7                    |
| 5          | 5                | 155         | 48            | 45.7        | 16.7                    |
| 6          | 10               | 156         | 49            | 43.6        | 14.6                    |

When the pitches prepared as above, by reaction with carbon tetrachloride, were subjected to coking temperatures, it was observed that loss due to volatility under coking conditions was about 2 per cent less when 1 per cent of carbon tetrachloride was employed than when coking

an untreated pitch. Even this slight increase in weight of non-volatile residue is of commercial importance when converted into terms of finished carbonized or graphitized articles. According to the above example, the use of 1 pound of carbon tetrachloride at a cost of very few cents gives an added 2 pounds of finished product at a market value of several times the carbon tetrachloride cost. Over an extended production period the manufacturing savings thus effected are very appreciable.

Several series of electrodes have been prepared according to the invention. The coke-pitch mixtures, containing from 15 to 27 per cent of pitch, were treated with carbon tetrachloride in the manner previously set forth and in amount varying up to about 10 per cent of carbon tetrachloride calculated on the weight of pitch.

The average properties of electrodes from three of these series of preparations is given in the following Table II, in comparison with the average of a similar number of electrodes of the same size (about 180 pounds each) made without the use of carbon tetrachloride.

Table II

| Group | Number of electrodes | Per cent carbon tetrachloride | Average resistance ohms/in. <sup>3</sup> | Average apparent density |
|-------|----------------------|-------------------------------|------------------------------------------|--------------------------|
| 1     | 15                   | 0                             | 0.000340                                 | 1.54                     |
| 2     | 3                    | 1                             | 0.000304                                 | 1.57                     |
| 3     | 6                    | 3                             | 0.000324                                 | 1.58                     |
| 4     | 3                    | 5                             | 0.000324                                 | 1.589                    |

The presence of carbon tetrachloride in the pitch-coke mixture not only makes for improved carbonized and graphitized articles, but, in spite of the higher melting point imparted to the pitch thereby, permits of the molding or extrusion of shaped articles at moderate working pressures of, for example, from 600 to 1200 pounds per square inch, such as are used when no carbon tetrachloride has been added to the mix.

The invention has been illustrated with respect to carbon tetrachloride as the polychlorinated hydrocarbon, and acetylene tetrachloride has been suggested as among the equivalents for carbon tetrachloride. The polychloro-hydrocarbon employed need not be a liquid such as those named above, as hexachloroethane and benzene hexachloride, both solids, have been found to exert an advantageous effect on the mixture and to yield graphitized articles of improved characteristics. These and many other polychloro-hydrocarbons, including chloroform, pentachloroethane, polychlorocyclohexane, and the like, have also been found to give the described reaction.

The present improvement relates as well to the manufacture from coke and pitch of articles wherein the pitch binder is merely carbonized as to those wherein both the binder and the coke are graphitized. It may be employed with advantage in the manufacture of shaped articles other than electrodes, and the compo-

sition is capable of being molded as well as extruded to form the improved products.

Other modes of applying the principle of our invention may be employed instead of the one explained, change being made as regards the method herein disclosed, provided the step or steps stated by any of the following claims or the equivalent of such stated step or steps be employed.

We therefore particularly point out and distinctly claim as our invention:

1. A method of treating pitch to increase the binding power thereof in coke-pitch mixtures which comprises heating pitch to a reaction temperature with a minor quantity of a polychlorinated hydrocarbon, and thereafter carbonizing the so-treated pitch in admixture with coke.

2. A method of treating pitch to increase the melting point, free carbon content and coking power thereof, and to increase its binding power in coke-pitch mixtures which comprises heating the pitch to a temperature above its melting point with from 0.7 to 6 per cent of its weight of carbon tetrachloride, and thereafter carbonizing the so-treated pitch in admixture with coke,

3. The method of making shaped articles from coke and pitch which comprises mixing finely divided coke and finely divided pitch with a minor quantity of a polychlorinated hydrocarbon, heating the mixture to a temperature above the initial melting point of the pitch but below a carbonizing temperature, shaping the resulting mixture, and heating the shaped article to carbonize the binder.

4. The method of making shaped articles from coke and pitch which comprises mixing from 73 to 85 parts of finely divided petroleum coke with correspondingly from 27 to 15 parts of finely divided coal-tar pitch and a minor quantity of carbon tetrachloride, heating the mixture to a temperature at which carbon tetrachloride reacts with pitch above the initial melting point of the pitch but below a carbonizing temperature, shaping the resulting mixture and heating the shaped article to carbonize the binder.

5. The method of making shaped articles from coke and pitch which comprises mixing from 73 to 85 parts of finely divided petroleum coke with correspondingly from 27 to 15 parts of finely divided coal-tar pitch and from 0.7 to 6 per cent, based on the pitch weight, of carbon tetrachloride, heating the mixture to a temperature at which carbon tetrachloride reacts with pitch above the initial melting point of the pitch but below a carbonizing temperature, shaping the resulting mixture and heating the shaped article to carbonize the binder.

6. The method as claimed in claim 4, wherein the baking is carried to graphitizing temperatures to graphitize both the coke and the binder, thereby to produce an article of higher apparent density and lower electrical resistance than have articles produced in like manner but without the carbon tetrachloride.

EDWARD R. COLE,  
RICHARD I. THRUNE.